

No. 802,493.

PATENTED OCT. 24, 1905

T. S. BLAIR, JR.  
PROCESS OF REDUCING METALLIC OXIDS  
APPLICATION FILED SEPT. 1, 1904.



Witnesses  
Forrest Smith  
C. H. Grisbauer

Inventor  
Thomas S. Blair, Jr.  
by *A. B. Willson*  
Attorney

# UNITED STATES PATENT OFFICE.

THOMAS SHOENBERGER BLAIR, JR., OF WOODMERE, NEW YORK,  
ASSIGNOR OF ONE-HALF TO B. C. LAUTH, OF PITTSBURG,  
PENNSYLVANIA.

## PROCESS OF REDUCING METALLIC OXIDS.

No. 802,493.

Specification of Letters Patent.

Patented Oct. 24, 1905.

Application filed September 1, 1904. Serial No. 223,037.

To all whom it may concern:

Be it known that I, THOMAS SHOENBERGER BLAIR, Jr., a citizen of the United States, residing at Woodmere, in the county of Nassau 5 and State of New York, have invented certain new and useful Improvements in Processes of Reducing Metallic Oxids; and I do declare the following to be a full, clear, and exact description of the invention, such as will enable 10 others skilled in the art to which it appertains to make and use the same.

My invention relates to improvements in processes for reducing metallic oxids mixed with gangue, especially iron oxids, whereby I 15 am enabled to economically produce wrought-iron direct from the ore and which is free from metalloids and is in condition for use, as hereinafter described and claimed.

In the accompanying drawings, Figure 1 is 20 an elevation of one form of furnace which may be used in carrying out my improved process. Fig. 2 is a sectional view of the same.

Referring to the drawings, which show one form of furnace that may be used in the operation 25 of my process, *a* is a steel or iron shell lined with suitable refractory material *b*, such as magnesite or chrome brick. This shell is supported on and revolved by the supporting-rollers *c*, which may be driven by any suitable 30 means. The furnace is provided with a removable connection *d* to a draft-flue *e*, which is connected with the chimney-stack (not shown) for the purpose of carrying off the products of combustion. This removable connection 35 also acts as a door through which the ore may be introduced into the furnace and the ball of metallic iron withdrawn from the furnace. The furnace is provided with a tap-hole *f*, which 40 enables the molten cinder to be discharged from the furnace. The latter is further provided with a door *g*, having an opening through which an oil or gas burner *h* projects for the purpose of introducing the reducing gas or atmosphere to the interior of 45 the furnace. The said door is also provided with an opening *i*, having a removable cover through which the operation of the furnace may be observed. This door is so constructed that it may be readily removed from the end 50 of the furnace, so that it also may be used for the introduction of the ore and the withdrawal of the metal in the form of a ball.

To enable my process to be carried on

largely and to provide for the economical charging and discharging of the furnace employed, I preferably build the furnaces side by side, with their ends in line, and employ an electric charging-machine, with charging-boxes, such as is in common use for charging open-hearth steel-melting furnaces operating 55 in front of one end of the furnace and adapted for charging the ore at such end of each furnace, and also employ a similar machine equipped with suitable tongs operating in front of the opposite end of the furnace for 60 the withdrawal of the iron balls.

The operation of my improved process is as follows: The metallic oxids to be reduced are finely ground, if not already in granular form, and are charged into the furnace, where they 65 are exposed to and enveloped in a reducing (deoxidizing) atmosphere, which may be obtained by the partial combustion of carbon or hydrocarbon gases introduced from the burner *g*. Coal, coal-gas, or oil may be used to produce 70 such gases and such reducing atmosphere. A sufficient quantity of the gases is burned to create a temperature of from 400° to 1,000° Fahrenheit, which is sufficient for the chemical reactions required for removal of the 75 oxygen from the metallic oxids, but leaving unconsumed a great proportion of the reducing agents, (carbon and hydrogen,) which having greater affinity than iron or other similar metals for oxygen decompose the metallic oxids at 80 such temperature and unite with the oxygen, the products of this combustion passing out of the furnace and leaving the iron or other metal treated practically free from all impurities. During this operation the furnace is mechanically 85 revolved or rotated, the effect being to expose the finely-divided particles of the metallic oxids to intimate and thorough contact with the heated reducing agents, insuring rapid and complete deoxidation and minimizing the 90 fuel consumption and also causing the iron or other metal to gather together in a ball similar to the ordinary puddle-ball as it parts with its oxygen and assumes the metallic form. When the oxygen has all been eliminated from chemical combination with the metal, the temperature in the furnace is increased by causing a more complete combustion 95 of the fuel, so as to melt the gangue or extraneous matter contained in the mineral 100 and burn out the metalloids, suitable fluxes;

- being added at this point of the operation, if desired or necessary, and the fused gangue or extraneous matter is then tapped off in the form of liquid cinders; but the temperature 5 is at no time raised sufficiently to fuse the metal, and the metallic ball when the liquid cinder has been separated therefrom is then removed from the furnace and constitutes a high quality of wrought-iron which is free 10 from metalloids and is in condition for use and may be delivered to the squeezer or hammer and rolls, like the ordinary puddle-ball, or may be used for melting stock for the open-hearth furnace or crucible.
- 15 It may be observed that I do not in carrying out my improved process employ a solid reducing agent, and hence am enabled to produce wrought-iron direct from the ore and without fusing the same, which would be 20 necessary, if a solid reducing agent were employed, in order to get rid of the particles of carbonaceous material which would become mechanically mixed with the metal.

Having thus described my invention, what I 25 claim as new, and desire to secure by Letters Patent, is—

1. The process of reducing metallic oxids mixed with gangue, consisting in removing the oxygen therefrom by subjecting the same 30 to contact with a reducing-gas at a temperature sufficient to cause the required chemical reactions, but with an insufficient supply of free oxygen to consume the reducing agents, changing the reducing temperature to a non- 35 reducing one by supplying more air, raising

the temperature sufficiently to fuse the gangue or extraneous matter and burn out the metalloids but not to the extent required to fuse the metal, separating the fused gangue or extraneous matter from the metal by melting 40 the gangue therefrom and balling the metal while the gangue is being melted away therefrom.

2. The process of reducing metallic oxids mixed with gangue, consisting in maintaining 45 a body of particles of such oxids in motion, to successively bring all of such particles to the surface, subjecting said moving body of such oxids to contact with a reducing-gas at such temperature as to cause the chemical 50 reactions required to remove the oxygen therefrom, but with an insufficient supply of free oxygen to consume the reducing agents, changing the reducing temperature to a non-reducing one by supplying more air, raising 55 the temperature sufficiently to fuse the gangue or extraneous matter and burn out the metalloids, but not to the extent required to fuse the metal, and while continuing to so move such body separating the fused gangue or extraneous matter from the metal, and balling the latter, substantially as described.

In testimony whereof I have hereunto set my hand in presence of two subscribing witnesses.

THOMAS SHOENBERGER BLAIR, JR.

Witnesses:

W. H. KANE,  
H. MICHAELIS.